

## UNITED STATES PATENT OFFICE

CHAD H. HUMPHRIES, OF INDIANAPOLIS, INDIANA, ASSIGNOR TO JAMES C. PATTEN, OF INDIANAPOLIS, INDIANA; E. KIRK MCKINNEY, SPECIAL ADMINISTRATOR OF SAID JAMES C. PATTEN, DECEASED

## COMPOSITION FOR CADMIUM PLATING BATHS

No Drawing.

Application filed October 1, 1928. Serial No. 309,694.

In my applications pending in the Patent Office, Serial Nos. 257,152, 267,273 and 221,619, I have described a certain type of plating bath which is acid and from which a fine, smooth, homogeneous, continuous coat of bright cadmium can be deposited.

It is the object of the present application to provide an improvement or a modification of the composition described in said above 10 mentioned applications.

Plating baths vary in composition and also in throwing power, which latter term is the platers' term covering the readiness or lack of readiness with which a metal from a given 15 solution tends to throw into recesses or deep holes. Some plating solutions have this throwing power property to a marked extent, while others, such as for instance, the average chromium plating solution has this 20 property to a very limited extent. The greater the throwing power of a plating solution, the more even is the deposit of the metal from such solution all over the surface of the article to be plated. Hence—the necessity 25 for improving the throwing power of any plating solution.

In this application now described, I have modified the formulae from that set forth in said applications with this point in view, 30 and have improved this type of acid cadmium plating bath.

In general, acid cadmium plating solutions do not have as high a throwing power as a cyanide plating solution of the same metal, 35 and in some cases are not employed to plate various articles, for that reason. In the bath of this application the throwing power is quite high. A suitable formula is now given for a still solution, per gallon of water

40 8 oz.  $H_2SO_4$  used  
4 oz.  $Al_2(SO_4)_3 \cdot 12H_2O$   
10 oz.  $Na_2SO_4 \cdot 10H_2O$  Present per gal.  
2.8 oz.  $CdO$  or 1 1/2 oz. free  $H_2SO_4$   
2.8 oz.  $Cd(OH)_2$  or  
3.1 oz.  $CdCO_3$   
10 g. glue

45 The bath using this formula can be made in one or two ways, and description is here given of two methods for making up a plating bath of this formula.

50 Add cadmium salt which can be hydrate, oxide or carbonate. Add to the above about

half a gallon of water, containing enough sulphuric acid to react with the cadmium salt, plus a definite amount of free sulphuric acid, which can be from 1/2 to 1 1/2 oz. per gallon. To another half gallon of water is added the other salts which can be sodium sulphate, ammonium sulphate or aluminum sulphate. The two are then mixed. After mixing, about a pint of this solution is removed and then there is dissolved the brightening agent, which can be glue, for example. This is done by heating this pint of solution and adding the glue and stirring. The solution containing the glue is then added to the remainder of the bath. The solution then contains the cadmium salt and some free acid and the other salts which act as agents for improving the throwing power, with the exception of the aluminum sulphate which is to tend to make a whiter deposit of cadmium. The glue acts as the brightening agent.

I do not limit myself to the use of glue alone as a brightening agent, but can use isinglass, agar agar or glucose.

75 When such a plating bath is used, cadmium anodes of the purity, such as is found in commercial cadmium is used, and the tank which holds the solution is preferably a wooden tank, which is lined with pitch and asphaltum.

80 Such a bath is self maintaining, though there may be a slight tendency for the metal content to increase, but slowly, in which case some anodes are removed from time to time, until the metal content becomes lower.

85 The above formula is suitable as mentioned for a still bath. When barrel plating is done, I prefer to use somewhat different concentrations, and below is given the formula for such a bath.

90 6.0 oz.  $H_2SO_4$   
6 oz.  $Al_2(SO_4)_3 \cdot 12H_2O$   
18. oz.  $Na_2SO_4 \cdot 10H_2O$   
8 oz.  $(NH_4)_2SO_4$  Present per gal.  
3.5 oz.  $Cd(OH)_2$  or 3.5 ozs. free  $H_2SO_4$ , approximately  
3.1 oz.  $CdO$  or  
3.5 oz.  $CdCO_3$   
10 g. glue

95 In place of using the above described method of making up such solution, I can if I wish, employ a mixture of the dry salts included in this formula, dissolving them in 100

hot water and stirring them. They are then readily soluble and form a constant composition. In making the bath initially, there is a tendency for some of the aluminum sulphate of commerce, to give the bath a milky appearance, but after using for a little time, this milky appearance disappears. During this milky period, there is a tendency for some of the glue to settle out, but after the 10 milkiness has disappeared this condition is not found.

Brightening agents of the types indicated have a tendency to slowly come out of the bath and be co-deposited with the cadmium, 15 but they can be added in lesser quantities than as shown in the formula, when evidence of their elimination is indicated by diminishing brightness.

It will be necessary from time to time to 20 scrub the anodes, as they become slightly filmed, particularly while standing. But this is not a great difficulty and is commercial plating room practice for other types of plating baths.

25 The solution in the still tank is operated at ordinary room temperature, which may mean between 60° F. and 90° F., but the solution in the barrel plating tank is apt to raise to higher temperature than this. Apparently temperatures of 120° F. and 130° F. 30 can be used without any harm to a barrel plating solution.

Current densities in the still baths are between 10 and 20 amperes per sq. ft., the usual 35 range being between 12 and 15 amperes per sq. ft. Above these current densities, there is a tendency for the color of the deposit to change and to become duller and if considerably higher current densities are used, 40 there will be treeing.

In barrel plating solutions, the barrel parts should not be made of iron or steel, as is sometimes used, but should be of brass, to prevent the dissolution of the iron in this solution.

45 Coats of desirable thickness for proper protection on iron and steel articles can be obtained in a smooth form from these solutions, which means thicknesses of from .0001 to .0005. Coats of .0002 give a salt spray test 50 of several hundred hours.

The bath which I have above described may be prepared in dry salts form for shipment to the plant, and as an aid in maintaining constancy of composition.

55 There can be some slight increase or decrease from the composition given for the three added salts, namely ammonium sulphate, aluminum sulphate and sodium sulphate.

60 There can also be some variation from the cadmium metal content and the free acid content indicated. I can for example vary the aluminum sulphate content from 2 to 8 oz.; sodium sulphate from 10 to 20 oz. and ammonium sulphate from 2 to 10 oz.

I claim as my invention:

1. A composition of matter adapted for use in forming an acid solution for the electrodeposition of cadmium consisting of substantially three ounces of sulphuric acid, two to eight ounces of aluminum sulphate, ten to twenty ounces of sodium sulphate, two to five ounces of cadmium salts containing oxygen and ten grams of a brightener. 70

2. A composition of matter adapted for use in forming an acid solution for the electrodeposition of cadmium consisting of substantially three ounces of sulphuric acid, two to eight ounces of aluminum sulphate, ten to twenty ounces of sodium sulphate, two to ten 80 ounces of ammonium sulphate, two to five ounces of cadmium salts containing oxygen and ten grams of a brightener. 75

3. A composition of matter adapted for use in forming an acid solution for the electrodeposition of cadmium consisting of substantially three ounces of sulphuric acid, two to eight ounces of aluminum sulphate, ten to twenty ounces of sodium sulphate, two to five 85 ounces of cadmium oxide, and ten grams of a brightener. 90

4. A composition of matter adapted for use in forming an acid solution for the electrodeposition of cadmium consisting of substantially three ounces of sulphuric acid, two to eight ounces of aluminum sulphate, ten to twenty ounces of sodium sulphate, two to ten 95 ounces of ammonium sulphate, two to five ounces of cadmium oxide and ten grams of a brightener. 100

In witness whereof, I have hereunto set my hand at Arlington, N. J., this 22nd day of September, A. D. one thousand nine hundred and twenty-eight.

CHAD H. HUMPHRIES. 105

110

115

120

125

130